

# United States Patent Office

2,990,334

Patented June 27, 1961

1

2,990,334

## GELATIN CAPSULES ENCLOSING A WATER-MISCIBLE VEHICLE

Dean M. Graham, Summit, N.J., assignor to The Upjohn Company, Kalamazoo, Mich., a corporation of Delaware

No Drawing. Filed June 29, 1959, Ser. No. 823,291  
3 Claims. (Cl. 167—83)

This invention relates to gelatin capsules and more particularly to gelatin capsules enclosing a water-miscible vehicle which is inert to gelatin and which inhibits the action of water on gelatin, a substance normally easily affected and readily dissolved by water.

The use of gelatin in forms commonly referred to as soft (plasticized) capsules and hard (unplasticized) capsules is well recognized. Soft gelatin capsules are one-piece sealed capsules enclosing the encapsulated components. They are made in various shapes and sizes. Hard gelatin capsules are usually composed of two parts, a cap and a body which are fitted together after the body has been filled with an appropriate component or components. They are also made in a wide variety of sizes. Both soft capsules and hard capsules can enclose a wide variety of components.

The inherent mutual affinity of water and gelatin has resulted in serious difficulties in the art of encapsulating components into either soft or hard capsules. Special precautions are required to keep the water content in said components and in any accompanying vehicle at the minimum. Otherwise the water exerts deleterious effects on the gelatin. In the case of soft capsules, water-immiscible oils are widely used as vehicles for the components to be encapsulated. In the case of hard capsules, the materials to be encapsulated must be dried to a minimum content of water prior to encapsulation. If special precautions to exclude water from the vehicle and the components are not followed carefully, both hard and soft capsules will break down during the encapsulation process. If the capsules do survive this process, storage after manufacture results in softening of the capsules, the appearance of small holes at the point of any contact between water and the gelatin shell of the capsule, the gradual loss of the acceptable elegant character of the capsules and even loss of the encapsulated components.

The aforesaid difficulties in the manufacture, storage, product elegance and use of soft and hard capsules have caused a long-felt need for a vehicle which is water-miscible, inert to gelatin and has a superior solubilizing and dispersing action on a wide variety of components to be encapsulated. A particularly acute difficulty arises in the use of soft capsules enclosing water-soluble components. Since oily vehicles are customarily used to carry the components, ready dispersion and solution of the said components does not occur in aqueous media due to retarding of dispersion by the oil. For example, after the oral ingestion of gelatin capsules for therapeutic purposes, the encapsulated components must normally become dissolved in the aqueous medium in the gastrointestinal tract before absorption can take place. The components in oily vehicles must be leached away from the oil by the aqueous medium before the absorption can occur. Moreover, the use of oily vehicles in which many of the components to be encapsulated are insoluble greatly hampers the practical manufacture of filled gelatin capsules. Many components must be encapsulated in larger capsules than would be necessary if a water-miscible vehicle with no adverse effects on gelatin were available. It has been found also that some oily vehicles, particularly those carrying suspended components, are very difficult to encapsulate because of high viscosity.

2

The present invention provides a sealed gelatin capsule enclosing a vehicle containing a water-miscible dioxolane compound having the formula



wherein R is a member of the class consisting of hydrogen, methyl and ethyl; R<sup>1</sup> is a member of the class consisting of hydrogen, methyl and ethyl; and R<sup>2</sup> is a member of the class consisting of hydrogen, methyl, carbinol and ethylo. The vehicle is inert to gelatin, is water-miscible, and possesses superior solubilizing and dispersing action on a wide variety of components. Since the vehicle inhibits the action of water and hygroscopic substances on gelatin, both water and hygroscopic substances, in addition to other components, can be carried in the vehicle.

The present invention obviates the use of oily vehicles as carriers for components to be encapsulated. Moreover, the capsule of the present invention provides ready dispersion of the encapsulated components upon contact of the capsule with an aqueous medium.

The inventive capsule encloses a vehicle containing a compound of the formula



wherein R is hydrogen, methyl or ethyl; R<sup>1</sup> is hydrogen, methyl or ethyl; and R<sup>2</sup> is hydrogen, methyl, carbinol or ethylo. The preferred compound is 2,2-dimethyl-4-carbinol-1,3-dioxolane. The other dioxolane compounds of this class, suitable in the vehicle, are

- 40 1,3-dioxolane,  
4-methyl-1,3-dioxolane,  
4-carbinol-1,3-dioxolane,  
4-ethylo-1,3-dioxolane,  
2,2-dimethyl-1,3-dioxolane,  
2,2,4-trimethyl-1,3-dioxolane,  
2,2-dimethyl-4-ethylo-1,3-dioxolane,  
2,2-diethyl-1,3-dioxolane,  
2,2-diethyl-4-methyl-1,3-dioxolane,  
2,2-diethyl-4-carbinol-1,3-dioxolane,  
2,2-diethyl-4-ethylo-1,3-dioxolane,  
2-methyl-1,3-dioxolane,  
2,4-dimethyl-1,3-dioxolane,  
2-methyl-4-carbinol-1,3-dioxolane,  
2-methyl-4-ethylo-1,3-dioxolane,  
2-ethyl-1,3-dioxolane,  
2-ethyl-4-methyl-1,3-dioxolane,  
2-ethyl-4-carbinol-1,3-dioxolane,  
2-ethyl-4-ethylo-1,3-dioxolane,  
2-ethyl-2-methyl-1,3-dioxolane,  
2,4-dimethyl-2-ethyl-1,3-dioxolane,  
2-ethyl-2-methyl-4-carbinol-1,3-dioxolane, and  
2-ethyl-2-methyl-4-ethylo-1,3-dioxolane.

The said vehicle is practically inert to gelatin. Further, it inhibits the action of hygroscopic components or substantial amounts of water on gelatin capsules. The affinity of any water present in the gelatin, in the diluted vehicle, or in the encapsulated components, for the vehicle is much greater than for the capsule. Thus, the capsule is protected from solution in, or softening by, the water, so that the capsule retains its shape during processing and its acceptable characteristics subsequent

to manufacturing. Moreover, the water-miscible nature of the vehicle furthers ready dispersion and solution in water of the encapsulated components.

The components are dissolved, suspended or emulsified in the vehicle by conventional means prior to encapsulation into the gelatin capsules. Encapsulation into the gelatin shells is carried out by means and methods known in the art. In the case of hard capsules, the known techniques for sealing the fitted body and cap can be utilized.

The dispersing and solubilizing properties of the vehicle of the invention are such that the vehicle can be used for the encapsulation of both liquid and solid components. The vehicle will dissolve both water-soluble and water-insoluble components. For example, flavors, perfumes, essences, foaming agents, surfactants, cosmetics, food products, vitamins and medicinals can be encapsulated by utilizing said vehicle.

Hard gelatin capsules and soft gelatin capsules were exposed to the action of a vehicle containing 2,2-dimethyl-4-carbinol-1,3-dioxolane to ascertain the effect on the gelatin of various concentrations of water present in the vehicle. The condition of the capsules was observed at various times and the observations recorded in Table I. The observations were made at 25 degrees centigrade.

TABLE I

25° C. stability of gelatin capsules in vehicle containing  
a vehicle containing  
2,2-dimethyl-4-carbinol-1,3-dioxolane

|                    | Percent of Water in the Vehicle |                     |                       |                       |                         |
|--------------------|---------------------------------|---------------------|-----------------------|-----------------------|-------------------------|
|                    | 0                               | 10                  | 20                    | 30                    | 40                      |
| Hard Capsules..... | Stable—<br>38 days.             | Stable—<br>38 days. | Softened—<br>4 hours. | Softened—<br>1½ hrs.  | Softened—<br>1 hour.    |
| Soft Capsules..... | do.....                         | do.....             | Swelled—<br>6 days.   | Swelled—<br>20 hours. | Dissolved—<br>48 hours. |

These data indicate that as much as ten percent water does not adversely affect either soft or hard gelatin capsules in the presence of the 2,2-dimethyl-4-carbinol-1,3-dioxolane.

The following examples set forth the best mode contemplated by the inventor of carrying out his invention but are not to be construed as limiting the invention.

## EXAMPLE 1

Soft gelatin capsules enclosing a vehicle containing aqueous lemon juice concentrate are prepared as follows:

Aqueous lemon juice concentrate ..... mls. 50  
2,2-dimethyl-4-carbinol-1,3-dioxolane ..... mls. 950

The two ingredients are well mixed and encapsulated by the usual techniques into soft capsules provided with a tip. The finished capsules do not soften or leak. At the time of use the tip is severed or punctured to facilitate expression of the capsule contents for flavoring.

## EXAMPLE 2

Soft gelatin capsules enclosing a vehicle containing choline chloride are prepared as follows:

Choline chloride ..... gms. 500  
Purified water, U.S.P. ..... mls. 40  
2-ethyl-2-methyl-1,3-dioxolane, q.s. ad ..... mls. 1000

The choline chloride is mixed with the water and the mixture stirred into the dioxolane. The whole is encapsulated by the usual techniques into 6.75 minim soft capsules. Each capsule encloses approximately 200 mg. of the choline chloride. The finished capsules do not soften or leak. The capsules are used in liver disorders such as fatty degeneration.

## EXAMPLE 3

Soft gelatin capsules enclosing a vehicle containing novobiocin are prepared as follows:

Novobiocin ..... gms. 700  
Purified water, U.S.P. ..... mls. 20  
2,2-dimethyl-4-carbinol-1,3-dioxolane, q.s. ad ..... mls. 1000

A solution of the novobiocin in the water and dioxolane is prepared and encapsulated by the usual techniques into 2.65 minim soft capsules. The finished capsules do not soften or leak. Each capsule provides approximately 1000 mg. of the medicament. The capsules are used orally in the treatment of staphylococcal infections.

## EXAMPLE 4

Soft gelatin capsules enclosing a vehicle containing an antiperspirant are prepared as follows:

Aluminum chlorhydroxide complex ..... gms. 20  
Purified water, U.S.P. ..... mls. 100  
2,2-dimethyl-4-ethylol-1,3-dioxolane, q.s. ad ..... mls. 1000

The aluminum chlorhydroxide is dissolved in the water. The solution is made up to volume with the dioxolane.

These data indicate that as much as ten percent water does not adversely affect either soft or hard gelatin capsules in the presence of the 2,2-dimethyl-4-carbinol-1,3-dioxolane and encapsulated by the usual techniques into 16 minim soft capsules provided with a tip. The finished capsules do not soften or leak. At the time of use the tip is severed or punctured to facilitate expression of the capsule contents.

## EXAMPLE 5

Sealed hard gelatin capsules enclosing a vehicle containing a vitamin mixture are prepared as follows:

Nicotinamide ..... gms. 2  
Vitamin B<sub>6</sub> hydrochloride ..... mgs. 50  
D-calcium pantothenate ..... mgs. 700  
Vitamin B<sub>1</sub> hydrochloride ..... mgs. 300  
Vitamin C ..... gms. 5  
Vitamin B<sub>2</sub> ..... mgs. 250  
Folic acid ..... mgs. 25  
Vitamin B<sub>12</sub> ..... mg. 0.250  
Ethanol ..... mgs. 39  
Vitamin A ..... units. 500,000  
Vitamin D ..... do. 50,000  
2-ethyl-2-methyl-4-carbinol-1,3-dioxolane, q.s. ad ..... minimis. 224

The well mixed ingredients are encapsulated by the usual techniques into hard capsules. The sealed finished capsules do not soften or leak. They are used in the oral treatment of vitamin deficiencies.

## EXAMPLE 6

Soft gelatin capsules enclosing a vehicle containing rose water are prepared as follows:

Rose water ..... mls. 400  
2-methyl-1,3-dioxolane ..... mls. 9600

The ingredients are well mixed and encapsulated by the usual techniques into soft capsules. The finished capsules do not soften or leak. At the time of use, the capsules are placed in water wherein rupture of the gelatin shell and dispersion of the capsule contents occur readily.

## EXAMPLE 7

Sealed hard gelatin capsules enclosing a vehicle containing a detergent are prepared as follows:

Sodium lauryl sulfate \_\_\_\_\_ gms. 5  
 Purified water, U.S.P. \_\_\_\_\_ mls. 7  
 2,2-dimethyl-4-carbinol-1,3-dioxolane, q.s. ad \_\_\_\_\_ mls. 100

A solution of the sodium lauryl sulfate in the water is prepared and made up to volume with the dioxolane. The whole is encapsulated by the usual techniques into hard gelatin capsules which are then sealed. The finished capsules do not soften or leak. At the time of use the capsules are placed in water wherein rupture of the gelatin shell and dispersion of the capsule contents occur readily.

It is to be understood that the invention is not to be limited to the exact details of operation or exact compositions shown and described herein as obvious modifications and equivalents will be apparent to one skilled in the art, and the invention is therefore to be limited only by the scope of the appended claims.

What is claimed is:

1. A sealed gelatin capsule enclosing a liquid water- 30

6  
 miscible vehicle containing (1) a water-miscible dioxolane compound having the formula



10 wherein R is a member of the class consisting of hydrogen, methyl and ethyl; R<sup>1</sup> is a member of the class consisting of hydrogen, methyl and ethyl; and R<sup>2</sup> is a member of the class consisting of hydrogen, methyl, carbinol and ethylol and (2) from 0 to about 10% of water based on the volume of said vehicle.

15 2. The capsule of claim 1 wherein the vehicle contains in addition a medicinal component.  
 3. The capsule of claim 1 wherein the vehicle contains in addition a vitamin component.

20

## References Cited in the file of this patent

## UNITED STATES PATENTS

2,667,268 Griffin \_\_\_\_\_ Jan. 26, 1954  
 2,872,377 Beiler \_\_\_\_\_ Feb. 3, 1959

## FOREIGN PATENTS

553,398 Canada \_\_\_\_\_ Feb. 18, 1958

## OTHER REFERENCES

Amer. Perfumer and Aromatics, February 1956, p. 25.